

## UNITED STATES PATENT OFFICE

2,520,108

## DYEING PROTEIN FIBERS WITH CHROMABLE ANTHRAQUINONE COLORS BY THE METACHROME PROCESS

Willard H. Watkins, Bound Brook, Henry E. Millson, Plainfield, and Chester A. Amick, Bound Brook, N. J., assignors to American Cyanamid Company, New York, N. Y., a corporation of Maine

No Drawing. Application July 18, 1947,  
Serial No. 761,982

14 Claims. (Cl. 8—30)

1

This invention relates to improvements in the metachrome dyeing process with chromable anthraquinone colors.

In the past, fibers such as wool, silk, synthetic protein fibers of similar type from casein, and the like have been dyed by the metachrome process in which the dyestuff and a mordant containing a chromium compound have been present in the dye-bath. In the dyeing procedure the dye is affixed to the fiber and is metallized. There have been many disadvantages to the metachrome dyeing process. For one thing, dye penetration has sometimes been inadequate because of premature reaction with the chromium containing mordant. Thus dyes which do not penetrate all of the fibers or are destroyed during the dyeing operation, particularly in the case of heavy shades, have been considered unsuitable for use in the metachrome process and have required resort to a process starting out with the preformed metallized dye or with a top or bottom chrome process. Among the chromable dyes which have been considered unsuitable for dyeing by the metachrome process are the chromable anthraquinone dyes and these dyes have, therefore, been excluded hitherto from metachrome dyeing.

Numerous attempts have been made to increase the penetration of the dyes and obtain stronger dyeings. One of the earlier attempts involved the use of cationic surface active agents. This process, however, did not achieve practical success because although greatly increased penetration resulted there was reaction between the surface active agent and the colored constituents of the dye-bath to produce a colored scum of precipitated dye and flocs. These larger colored aggregates often caused serious spots or flocs in the dyeing and precluded the practical use of this method. The next development which was practically useful involved the addition to the metachrome dye-bath of both cationic and nonionic surface active agents, the latter serving to keep the reaction products of the cationic agent and colored constituents in fine dispersion. This process forms the subject matter of the application of Millson and Royer, Serial No. 420,504, filed November 26, 1941, now abandoned.

It was later found by Royer and Amick (application Serial No. 542,445, filed June 27, 1944 now Patent No. 2,434,178) that if the cationic agent was colloidized, either alone or in conjunction with the chromable color or the mordant, increased penetration and level dyeing could be obtained without the presence of a nonionic surface agent.

2

In the earlier application Ser. No. 750,886, filed May 27, 1947, we have described and claimed a metachrome process in which the colloidized cationic surface active agent is associated with the other features. The first is the presence of a salt of an alkaline earth metal such as magnesium sulfate and secondly a procedure in which the dye bath initially has a pH sufficiently high so that rapid chromation is prevented or retarded and the pH is then progressively lowered by boiling until final chromation results.

According to the present invention we have found that with certain chromable anthraquinone colors a marked increase in color strength is obtained if the alkaline earth metal salt and initial high pH followed by a reduced pH is used without any cationic surface active agent. The alkaline earth metal salt in the present case as in the earlier application above referred to must of course have an anion which does not form complexes with chromium containing salts. The increase in strength is marked and there is no problem of scum formation. It is thus possible to obtain strengths which do not compare unfavorably with those obtained by the process of the co-pending application above referred to without requiring any cationic agent and hence encountering no problem of colored scum or floc formation.

It is not known why with chromable anthraquinone colors the marked increase in strength is obtained without any cationic surface active agent. This is not generally true because with many chromable colors of other types the cationic surface active agent is essential. It is possible that the mechanism of dyeing the chromable anthraquinone colors by a metachrome process may differ somewhat from the dyeing mechanism of some other chromable colors and it is not desired to limit the present invention to any theory of dyeing mechanism.

The invention will be described in conjunction with the following specific examples. The parts are by weight.

## Example 1

45 A dye bath is prepared comprising 2% of the dye having Color Index No. 1085, 10% ammonium sulfate and 1% potassium bichromate in 400 ml. of distilled water. A 5-g. woolen skein or piece, 50 pre-wet with distilled water, is entered into the dye bath which is gradually heated to the boil in about 30 minutes. The bath is then boiled for about 30 minutes, after which the volume of water is replenished and 2% of 28% acetic acid is added. Boiling is continued for another 30 minutes,

the water again replenished and 4% of 28% acetic acid is added. Boiling is again continued for about 30 minutes after which the dyed wool is removed, rinsed in distilled water, squeezed and dried. During the dyeing the wool is turned intermittently to obtain penetration of maximum uniformity. This is a "control" dyeing and the procedure used is one that is often recommended for dyeing chromable colors by the metachrome process. All the above percentages are based on 10 the weight of the wool.

A second dye bath is prepared comprising 2% of the same dye, 2% ammonium hydroxide to give a pH of about 9, 10% magnesium sulfate containing 7 molecules of water of crystallization and 0.6% potassium bichromate in 400 ml. of distilled water. A 5-gram wool sample is entered into this bath and dyed as above. The color value of the two samples is then determined by means of a spectrophotometer. If the value of the control 20 is 100%, then the wool dyed in the solution containing the ammonium hydroxide and the magnesium sulfate has a value of 116%.

*Example 2*

The procedure of the preceding example is followed exactly except the dye having Color Index 1034 is used instead of the dye having Color Index 1085. When the control dyeing is given a value of 100%, then the wool dyed in the bath 30 containing the ammonium hydroxide and the magnesium sulfate is 109%.

*Example 3*

The procedure of Example 1 is repeated exactly except 10% of calcium nitrate is used instead of 10% of the magnesium sulfate of Example 1. When the control dyeing is assigned a value of 100%, the skein dyed in the dyebath containing the calcium nitrate and ammonium hydroxide has a color value of 118%.

*Example 4*

The procedure of Example 1 is repeated exactly except 10% strontium nitrate is used instead of the magnesium sulfate of Example 1. When the control dyeing is assigned a value of 100%, the wool dyed in the presence of the strontium salt and ammonium hydroxide has a value of 116%.

We claim:

1. A method of dyeing which comprises subjecting substantially unmetallized protein fibers to the action of a dye bath formed by mixing a chromable anthraquinone dye, a soluble alkaline earth metal salt the anion of which does not form complexes with chromium containing salts, a soluble chromium containing salt, water, and sufficient alkali to make the bath alkaline and to cause said dye to react with said alkaline earth metal salt to form an alkaline earth metal complex of said dye and insufficient to materially damage said fibers, partially dyeing said fibers from said complex, gradually lowering the pH of said bath to a point where decomposition of said complex and chromation of the dye take place, and completing the dyeing at said lowered pH.

2. A method of dyeing which comprises subjecting substantially unmetallized protein fibers to the action of a dye bath formed by mixing a chromable anthraquinone dye, a soluble chromium containing salt, magnesium sulfate, water, and sufficient alkali to make the bath alkaline and to cause said dye to react with said alkaline earth metal salt to form an alkaline earth metal com-

plex of said dye and insufficient to materially damage said fibers, partially dyeing said fibers from said complex, gradually lowering the pH of said bath to a point where decomposition of said complex and chromation of the dye take place, and completing the dyeing at said lowered pH.

3. A method of dyeing which comprises subjecting substantially unmetallized wool fibers to the action of a dye bath formed by mixing a chromable anthraquinone dye, a soluble alkaline earth metal salt the anion of which does not form complexes with chromium containing salts, a soluble chromium containing salt, water, and sufficient alkali to make the bath alkaline and to cause said dye to react with said alkaline earth metal salt to form an alkaline earth metal complex of said dye and insufficient to materially damage said fibers, partially dyeing said fibers from said complex, gradually lowering the pH of said bath to a point where decomposition of said complex and chromation of the dye take place, and completing the dyeing at said lowered pH.

4. A method of dyeing which comprises subjecting substantially unmetallized wool fibers to the action of a dye bath formed by mixing a chromable anthraquinone dye, a soluble chromium containing salt, magnesium sulfate, water, and sufficient alkali to make the bath alkaline and to cause said dye to react with said alkaline earth metal salt to form an alkaline earth metal complex of said dye and insufficient to materially damage said fibers, partially dyeing said fibers from said complex, gradually lowering the pH of said bath to a point where decomposition of said complex and chromation of the dye take place, and completing the dyeing at said lowered pH.

5. A method of dyeing which comprises subjecting substantially unmetallized wool fibers to the action of a dye bath formed by mixing a chromable anthraquinone dye, a soluble alkaline earth metal salt the anion of which does not form complexes with chromium containing salts, a soluble chromium containing salt, water, and sufficient alkali to make the bath alkaline, but with a pH not greater than 9.5, and to cause said dye to react with said alkaline earth metal salt to form an alkaline earth metal complex of said dye and insufficient to materially damage said fibers, partially dyeing said fibers from said complex, gradually lowering the pH of said bath to a point where decomposition of said complex and chromation of the dye take place, and completing the dyeing at said lowered pH.

6. A method of dyeing which comprises subjecting substantially unmetallized wool fibers to the action of a dye bath formed by mixing a chromable anthraquinone dye, a soluble chromium containing salt, magnesium sulfate, water, and sufficient alkali to make the bath alkaline, but with a pH not greater than 9.5, and to cause said dye to react with said alkaline earth metal salt to form an alkaline earth metal complex of said dye and insufficient to materially damage said fibers, partially dyeing said fibers from said complex, gradually lowering the pH of said bath to a point where decomposition of said complex and chromation of the dye take place, and completing the dyeing at said lowered pH.

7. A method according to claim 5 in which the anthraquinone dye is dye No. 1085 of the Color Index.

8. A method according to claim 5 in which the anthraquinone dye is dye No. 1034 of the Color Index.

9. A method according to claim 1 in which the pH of the dye bath is lowered by the addition of successive small portions of acid.

10. A method according to claim 2 in which the pH of the dye bath is lowered by the addition of successive small portions of acid.

11. A method according to claim 3 in which the pH of the dye bath is lowered by the additions of successive small portions of acid.

12. A method according to claim 4 in which the pH of the dye bath is lowered by the additions of successive small portions of acid.

13. A method according to claim 5 in which the pH of the dye bath is lowered by the additions of successive small portions of acid.

14. A method according to claim 6 in which the pH of the dye bath is lowered by the additions of successive small portions of acid.

WILLARD H. WATKINS.  
HENRY E. MILLSON.  
CHESTER A. AMICK.

## REFERENCES CITED

The following references are of record in the file of this patent:

## UNITED STATES PATENTS

| Number    | Name    | Date          |
|-----------|---------|---------------|
| 941,399   | Winslow | Nov. 30, 1909 |
| 1,511,359 | Onnertz | Oct. 14, 1924 |
| 1,937,531 | Rogers  | Dec. 5, 1933  |
| 2,434,178 | Royer   | Jan. 6, 1948  |

## OTHER REFERENCES

"Theory and Practice of Wool Dyeing," by C. L. Bird, published 1947 in London by the Society of Dyers and Colorists, pages 87, 88.

"Application of Coal Tar Dyestuffs," by C. M. Whittaker, published 1919 in London by Bailliere, Tindall and Cox, pages 59-61, inclusive.

"Application of Dyestuffs," by J. M. Matthews, published in New York by John Wiley & Sons, 1920. Pages 356-358.

"Metachrome Method of Dyeing," by C. H. A. Schmitt, article in Amer. Dyes Reporter for June 26, 1939, pp. P336-P341.